

March 24, 1970

H. KRÄSSIG ET AL  
TREATMENT OF TEXTILE MATERIALS WITH  
RADIATION AND CAUSTIC ALKALI

3,502,426

Filed March 3, 1965

2 Sheets-Sheet 1

Sodium Hypoxide Solutions

15-22°C



Fig. 1.

Fig. 2.

INVENTORS

BY  
HANS KRÄSSIG  
FRITZ MÜNZEL  
HANS-JOERG SCHENKEL

Ward, Haskins, McElhenny, Erman, Brooks & Lyle, Patrick  
ATTORNEYS

March 24, 1970

H. KRÄSSIG ET AL  
TREATMENT OF TEXTILE MATERIALS WITH  
RADIATION AND CAUSTIC ALKALI

3,502,426

Filed March 3, 1965

2 Sheets-Sheet 2

Potassium Hydroxide Solutions



INVENTORS  
HANS KRÄSSIG  
FRITZ MÜNZEL  
BY HANS JOERG SCHENKEL

May, Hulbert, McElroy, June, Broder & Litschick  
ATTORNEYS

## 1

3,502,426

TREATMENT OF TEXTILE MATERIALS WITH  
RADIATION AND CAUSTIC ALKALI

Hans Krässig, Fritz Münz, and Hans-Joerg Schenkel,  
Schwerzenbach, Switzerland, assignors to Heberlein  
Patent Corporation, New York, N.Y., a corporation  
of New York

Filed Mar. 3, 1965, Ser. No. 436,810

Claims priority, application Switzerland, Mar. 13, 1964,

3,272/64

Int. Cl. D06m 1/00

U.S. Cl. 8—116

8 Claims

This invention relates to the treatment of fabrics, and more particularly, it relates to a process for the removal of radiation energy from irradiated cellulosic textile materials.

For purposes of this application the terms "textile material" or "fabric" shall both be understood to include fabrics and textile materials of all kinds, including fibers, 20 yarns, threads, and any manner of knit or woven fabrics, as well as non-woven or felted fabrics. Further, for purposes of this application the term "cellulosic textile material" shall be understood to include fabrics of all kinds which consist entirely of natural and/or regenerated cellulose and mixtures thereof as well as all manner of fabrics, 25 films, or sheets in which such cellulosic constituents make up a significant portion thereof.

A number of processes to improve the wearing qualities of cellulosic fabrics by subjecting such fabrics of ionizing radiation are known in the art. Thus, cellulosic textile materials have been subjected to electromagnetic radiation, such as gamma rays emanating from radio-isotopes such as  $\text{Co}^{60}$  or  $\text{Cs}^{137}$ , X-rays, ultraviolet rays, and the like or by the use of particulates ionizing radiation such as electrons accelerated in cascade, Van de Graaf, and linear accelerators and the like or by Tesla transformers. Such irradiation of fabrics is believed to produce ions, ion radicals, free radicals, or activated molecules or groups of molecules which are capable of forming sites for cross-linking between atoms comprising the molecule, as disclosed in copending application Ser. No. 111,900. Such irradiation also fosters grafting reactions, especially in the case of monomeric substances which are capable of being polymerized or the graftable polymers disclosed in copending application Ser. No. 125,088.

Such irradiation of textile materials results in the accumulation of absorbed radiation energy in the fabric. While some of this energy is consumed in cross-linking and grafting reactions, the absorbed radiation energy is not and apparently cannot be completely utilized, probably because some of it is localized in areas of the structure, such as crystalline areas, which are inaccessible to the grafting chemicals or because some of the absorbed energy is present in a form which is not suitable for grafting or cross-linking reactions between the molecules. This energy which is present in the irradiated textile material and which cannot be utilized for cross-linking or grafting is designated herein as residual energy.

The residual energy remaining in the material may be very persistent and enduring. Some of the areas which have been activated by irradiation may have a long life and the textile material may retain the residual energy for a long time. Moreover, this residual or stored energy does not remain quiescent or inactive in the material, but in many cases it effects gradual changes in the physical properties, mechanical strength, and so on of the material.

## 2

Naturally, such subsequent changes in the properties of the treated irradiated fabric are undesirable. Moreover, there is the possibility of undesirable physiological effects from such residual or stored energy on the users of the fabrics. Such untoward effects would be most likely to occur in areas where the fabric directly contacts the skin of the wearer or user of artifacts made from irradiated materials.

This invention provides a process for the removal of residual energy from irradiated cellulosic textile materials.

Briefly, the process of this invention comprises treating a cellulosic textile material, which material has been subjected to ionizing radiation, in an alkaline bath containing an alkali-metal hydroxide at strengths above those normally used for mercerization.

It has been found that while the usual mercerization with a lye has little or no effect in the removal of the excess or residual radiation energy, surprisingly when the concentration of the lye is increased such residual energy is removed from the textile material. The process of this invention can be utilized in conjunction with cross-linking or grafting reactions of the material effected by means of ionizing radiation. The process has wide application to cellulosic textile materials, as the term is used herein, as for example to natural or native cellulose materials such as cotton and to regenerated cellulose materials such as viscose rayon or cuprammonium rayon.

The process of this invention and its application to the treatment of cellulosic materials can be more readily understood by reference to

FIGURES 1 and 2 which are graphic presentations of the results of treating irradiated cellulosic textile materials with sodium hydroxide solutions and

FIGURES 3 and 4 which are graphic representations of action of potassium hydroxide solutions on irradiated cellulosic textile materials.

The process of this invention is carried out with a solution of alkali-metal hydroxide stronger than those generally used for mercerization. For reasons of convenience and economy, it is generally preferred to use sodium hydroxide or potassium hydroxide, although mixtures of these or other alkali-metal hydroxides can also be used. Preferably, natural or native cellulose is treated in a bath containing alkali-metal hydroxide at a normality of from about 4 to about 9. This corresponds to a sodium hydroxide concentration of from about 14° to about 34° Bé, or potassium hydroxide concentrations of from about 22° to about 39° Bé. Regenerated cellulose materials are preferably treated in baths containing from about 2.5 to about 5 N alkali-metal hydroxide, this corresponding to a sodium hydroxide strength of from about 13° to about 23° Bé, or a potassium hydroxide strength of from about 15° to about 26° Bé.

The time of treatment required to remove the residual energy can be varied over wide limits. It is generally preferred that the treatment be carried out for from about 5 to about 20 minutes, the optimum time of treatment being interrelated with the temperature of treatment as more fully discussed hereinafter.

It is preferred that where the cellulosic textile material predominantly contains natural cellulose it be treated in a bath containing from about 8 to about 8.5 N alkali-metal hydroxide at a temperature on the order of 60° C. for from about 5 to about 10 minutes. Similarly, when the cellulosic textile material contains regenerated cellulose it is preferred to treat it with a 3.5 N

(17 Bé.) sodium hydroxide at from about 15 to about 25° C. for from about 5 to about 10 minutes.

The mutual interrelationship of hydroxide concentration and temperature of treatment for sodium hydroxide and potassium hydroxide used can be readily appreciated from the graphical representations presented in FIGURES 1 through 4. The data presented on these graphs represents the results of treating an imitation cotton poplin fabric which had been subjected to  $\text{Co}^{60}$  gamma radiation for 10 hours. The abscissas represent the deactivation time, that is, the time of treatment in the alkali-metal hydroxide, and the ordinates represent a measure of the residual energy remaining in the textile material. The amount of residual energy is shown as the magnitude or height of signal obtained from an electron-spin resonance (ESR) determination on the fabric.

Such means of ascertaining the residual energy left after irradiation of the textile material and any subsequent cross-linking or grafting operation depends upon the fact that an unpaired electron has a detectable magnetic moment. It has been found that this magnetic moment due to the so-called spin of the unpaired electron provides a measure of the residual energy remaining in the material after irradiation and subsequent operations. As is well-known to those skilled in the art the ESR can be determined by a number of methods, one of the most sensitive and most accurate being the determination of the microwave band absorption spectrum of the material under an applied magnetic field. The details of such methods are discussed at length in reference works such as D. J. E. Ingram, *Free Radicals as Studied by Electron Spin Resonance*, New York, Academic Press, 1958.

FIGURE 1 illustrates the removal of residual energy from the aforesaid cotton cellulosic textile material when it is treated at 60° C. with sodium hydroxide. This shows that with 8 N (31° Bé.) sodium hydroxide the residual radiation energy is completely eliminated after a 10-minute period. When 6 N (26° Bé.) sodium hydroxide is used, a substantial diminution of residual energy is obtained after 60 minutes of treatment. Similarly, FIGURE 2 shows the results obtained with 6 and 8 N sodium hydroxide at room temperature of 15° to 20° C. In this case, once again the 8 N sodium hydroxide has completely removed all residual radiation energy after 10 minutes.

In the same manner, FIGURES 3 and 4 show the results obtained when the treatment of this invention is carried out with potassium hydroxide at 8.5 (37° Bé.), 7 N (32° Bé.), and 5.5 N (27° Bé.) at the indicated temperatures. When the treatment is conducted at 60° C. a 8.5 N potassium hydroxide solution removes all residual radiation energy after 10 minutes. In FIGURE 4 where a room temperature of 15-22° C. is used, residual energy is completely eliminated from the cellulosic textile material after a 120-minute treatment with 8.5 N potassium hydroxide.

The following examples are set out to illustrate specific embodiments of this invention, and are not indicative of the entire scope of such invention, the scope being determined by the claims appended hereto.

#### EXAMPLE I

An imitation cotton poplin fabric having a moisture content of 5% (in other words the moisture content in equilibrium with the ambient room air) was irradiated with gamma rays from a  $\text{Co}^{60}$  source for 10 hours to obtain a total dose of  $2.2 \times 10^6$  rad. Subsequent to this irradiation the cellulose textile material was tested and found to have a relative ESR signal magnitude of 130 units.

Subsequently the textile material was treated for 10 minutes in a bath containing 8 N sodium hydroxide (about 31° Bé.) at 15-22° C. A sample was then rinsed with water, treated with dilute acetic acid, washed to a

neutral reaction, and dried. The textile material was once again tested for residual energy and no ESR signal could be detected. The residual radiation energy had been completely removed by this treatment. The process as shown by this example is applicable to other native cellulose materials with comparable results.

#### EXAMPLE II

A viscose rayon having a moisture content of 7% was irradiated with gamma radiation from a  $\text{Co}^{60}$  source for 10 hours to produce a total dose of  $2.2 \times 10^6$  rad. The material was then subjected to an ESR measurement which indicated a signal magnitude of 230 units.

The textile was then treated for 10 minutes at 60° with 8.5 N potassium hydroxide (37° Bé.). This material was then washed with water and acetic acid and dried as in Example I. When subsequently tested for ESR, no signal was obtained. Thus, the residual radiation energy was completely removed from the viscose rayon by the treatment.

The process of this example is applicable to other regenerated cellulose textile materials with comparable results.

It will be understood that cross-linking or grafting or other operations can take place between the irradiation and the elimination of excess or residual energy by the process of this invention. Further, the other well-known alkali-metal hydroxides can be used in this process, although the sodium and potassium hydroxides are preferred because of availability and economy.

What is claimed is:

1. A process for removing excess energy which comprises subjecting a cellulosic textile material selected from the group consisting of native cellulose and regenerated cellulose to ionizing radiation in an amount not greater than about  $10^7$  rad and treating the irradiated textile material for from about five to about twenty minutes in an aqueous alkaline bath containing from about 4 to about 9 N alkali-metal hydroxide when said material is native cellulose and from about 2.5 to about 5 N alkali-metal hydroxide when said material is regenerated cellulose.

2. The process of claim 1 wherein the alkaline bath is at a temperature in the range of from about 10° to about 30° C.

3. The process of claim 1 wherein the alkaline bath is at a temperature in the range of from about 50° to about 100° C.

4. A process for removing excess energy which comprises subjecting a textile material containing natural cellulose to an amount of ionizing radiation not greater than about  $10^7$  rad to introduce residual energy into said material and subsequently treating said material in a bath at about 60° C. for from about 5 to about 10 minutes, said bath containing from about 8 to about 8.5 N alkali-metal hydroxide.

5. The process of claim 4 wherein the alkali-metal hydroxide is sodium hydroxide.

6. A process for removing excess energy from a textile material which comprises subjecting a textile material containing regenerated cellulose to an amount of ionizing radiation not greater than  $10^7$  rad and subsequently treating said material in a bath at a temperature of from about 15° to about 25° C. for from about 5 to about 10 minutes, said bath containing about 3.5 N alkali metal hydroxide.

7. The process of claim 6 wherein the alkali-metal hydroxide is sodium hydroxide.

8. A process for removing excess energy which comprises treating a cellulosic textile material selected from the group consisting of native cellulose and regenerated cellulose, said material having been subjected to ionizing radiation in an amount not greater than about  $10^7$  rad which introduced residual energy into said material, in an aqueous alkaline bath containing from about 4 to about

9 N alkali-metal hydroxide when said material is native cellulose and from about 2.5 to about 5 N alkali-metal hydroxide when the material is regenerated cellulose, removing said material from said bath, and subsequently neutralizing any residual alkalinity in said material.

## OTHER REFERENCES

- R. H. Peters, "Textile Chemistry," vol. 11, Elsevier Publishing Co., New York, 1967, pp. 328, 329, 330, 333, 334.
- 5 NORMAN G. TORCHIN, Primary Examiner  
J. C. CALLAGHAN, Assistant Examiner

## References Cited

## UNITED STATES PATENTS

- |           |         |        |       |           |    |           |
|-----------|---------|--------|-------|-----------|----|-----------|
| 3,206,273 | 9/1965  | Munzel | ----- | 8—116     | 10 | 204—160.1 |
| 3,108,890 | 10/1963 | Beaver | ----- | 204—160.1 |    |           |

U.S. Cl. X.R.

UNITED STATES PATENT OFFICE  
CERTIFICATE OF CORRECTION

Patent No. 3,502,426 Dated March 24, 1970

Inventor(s) H. KRÄSSIG ET AL

It is certified that error appears in the above-identified patent and that said Letters Patent are hereby corrected as shown below:

Column 1, lines 5, 6 and 7 delete "to Heberlein Patent Corporation, New York, N.Y., a corporation of New York" and insert in lieu thereof --, by mesne assignments, to Heberlein & Co. A.G., Wattwil, St. Gall, Switzerland, a corporation of Switzerland --.

SIGNED AND  
SEALED

  
**OCT 27 1970**

(SEAL)

Attest:

**Edward M. Fletcher, Jr.**

Attesting Officer

**WILLIAM E. SCHUYLER, JR.**  
Commissioner of Patents